

Feb. 16, 1954

W. L. FINLAY ET AL

2,669,514

TITANIUM BASE ALLOYS CONTAINING TIN

Filed March 11, 1953

2 Sheets-Sheet 1

Fig. 1a.



Fig. 1b.



EFFECT OF ATMOSPHERE ON THE SCALING RATE

OF Ti AND Ti-Sn ALLOYS AFTER 4 HOURS. INVENTORS.

AT 1050°C.

WALTER L. FINLAY.

ROBERT I. JAFFEE.

HORACE R. OGDEN.

Ward Crosby & Real.

ATTORNEYS.

Feb. 16, 1954

W. L. FINLAY ET AL

2,669,514

TITANIUM BASE ALLOYS CONTAINING TIN

Filed March 11, 1953

2 Sheets-Sheet 2



Fig. 4a.

Fig. 5a.



Fig. 4b.

Fig. 5b.



Fig. 4c.

Fig. 5c.



Fig. 4d.

Fig. 5d.



Fig. 4e.

Fig. 5e.

INVENTORS.  
WALTER L. FINLAY.  
ROBERT I. JAFFEE.  
HORACE R. OGDEN.

BY

Ward Crosby & Neal

ATTORNEYS.

— — — VHN AFTER  $O_2$ ,  $N_2$  OR AIR TREATMENT METAL LOST BY SCALING WEIGHT GAIN ( $g/cm^2$ )  
EFFECT OF ATMOSPHERE ON SCALING BEHAVIOR AND CONTAMINATION RESISTANCE OF Ti AND Ti-SN ALLOYS  
HELD FOUR HOURS AT 1050°C AND FURNACE COOLED

## UNITED STATES PATENT OFFICE

2,669,514

## TITANIUM BASE ALLOYS CONTAINING TIN

Walter L. Finlay, Beaver, Pa., and Robert L. Jaffee, Worthington, and Horace R. Ogden, Columbus, Ohio, assignors, by direct and mesne assignments, to Rem-Cru Titanium, Inc., Midland, Pa., a corporation of Pennsylvania

Application March 11, 1953, Serial No. 341,796

6 Claims. (Cl. 75—177)

1

This invention pertains to titanium base alloys, and more particularly to strong, ductile and contamination resistant alloys of titanium and tin, which may optionally and beneficially contain relatively large and controlled amounts of one or more of the interstitials carbon, oxygen and nitrogen for further strengthening the same, while retaining therein adequate ductility for fabrication purposes, such as forging or rolling or otherwise plastically deforming.

This application is a continuation-in-part of our copending application Serial No. 222,938, filed April 25, 1951, now forfeited.

The strong and ductile titanium-tin alloys of the invention contain, according to the broad range of analysis, about 1 to 23% tin, although for tin contents below about 5% and particularly below about 2.5%, they require substantial additions of one or more of the interstitials carbon, oxygen and nitrogen or other alloying elements for materially enhancing the tensile properties as compared to the unalloyed and substantially uncontaminated titanium base metal.

The presence of tin alloyed with the titanium base metal greatly enhances the tolerance with respect to the interstitials carbon, oxygen and nitrogen without undue embrittlement and with resultant marked strengthening of the alloy. The carbon may range as high as about 1%, oxygen up to about 0.5%, and nitrogen up to about 0.3%.

For imparting a high degree of contamination resistance, i. e. resistance against diffusion into the alloy of atmospheric gases, particularly oxygen and nitrogen, at elevated temperatures up to about 1100° C., the alloy should contain upwards of about 5% tin, although lesser amounts down to about 2% tin are materially beneficial in this respect. Tin alloyed with titanium base metal appears to be unique in imparting this contamination resistance, and its effect is quite critical with respect to the degree of contamination resistance imparted commencing at a minimum of about 5% tin.

The alloys of the invention are also characterized by free scaling properties resulting from exposure to elevated temperatures up to about 1100° C. under atmospheric, oxidizing or alternatively oxidizing and reducing conditions. That is to say the scale formed is easily brushed off or

2

flakes off during hot forming such as forging or rolling. This is particularly true within the range of about 8 to 16% tin, the optimum effect in this respect occurring over the range of about 10 to 14% tin.

For tin contents up to about 16% these alloys also possess excellent welding characteristics, undergoing no appreciable loss of ductility in the welded as compared to the non-welded portions.

10 Substantially pure titanium may be produced at considerable expense by the Van Arkel or "iodide" process described in Patent 1,671,213. Other methods of production, such as the magnesium reduction of titanium tetrachloride, as described in the Patent 2,205,854 to Kroll, result in a metal of commercial purity containing traces of other metals, such as iron, and quantities of the interstitial constituents, carbon, nitrogen and/or oxygen, which in the range upwardly 15 from 0.01% may be significant. These contaminants have the effect of strengthening the metal but they tend to cause embrittlement. A combination of acceptable strength and ductility is difficult to achieve. Further strengthening has 20 hitherto been secured by the addition of varying quantities of a variety of other metals, but in general it has been found necessary to use as a base for such alloys, a titanium metal in which the total contaminant content was quite low. 25 The effect of the three contaminants is substantially additive. Nitrogen is the most potent hardener and strengthener, but ordinarily causes the greatest embrittlement. The strengthening effect of oxygen is usually less than that 30 of nitrogen, while soluble carbon is desirable, but any excess tends to form embrittling carbides.

35 The present invention comprises, in one of its aspects, the discovery of a group of binary alloys of titanium and tin which have desirable properties, and the further discovery that such alloys will not only tolerate carbon, oxygen and/or nitrogen, in quantities heretofore wholly unusable, but that the presence of one or more of these materials results in greatly augmented 40 strength at a high level of ductility. It has likewise been found that alloys of this group are not susceptible to deep and damaging penetration by atmospheric gases at fabricating temperatures.

45 Tin is soluble in alpha titanium to the extent of at least 15%, and alloys of titanium with up to

15% tin are all in the alpha phase. As the tin content is increased the beta transformation temperature rises, and at a temperature of about 930° C., and a tin content of about 19% a peritectoid reaction occurs. In alloys containing 20% to 23% tin, two intermediate phases have been tentatively identified.

An alloy containing about 5% tin, balance high purity or "iodide" titanium, as rolled and annealed for 2 hours at 850° C., has an ultimate strength of 64,000 p. s. i., an elongation in 1" of 18%, and a bend ductility of about 2.8 T. Increasing the proportion of tin substantially increases strength with only a relatively minor effect on ductility. As the tin content is increased, recrystallization by annealing after rolling becomes more difficult, but can be achieved by more extensive annealing. For example, an alloy containing about 17.5% tin, balance substantially pure titanium, after annealing for 24 hours at 850° C., has an ultimate strength of 111,000 p. s. i., an elongation in 1" of 19%, and a bend ductility

of 2.5 T. It will be seen that, as compared with the 5% tin alloy, strength has nearly doubled, while ductility, instead of decreasing in proportion to the increase in strength, is actually slightly improved. A further increase in tin content results in further strengthening with only a minor reduction in elongation and an apparent further improvement in bend ductility. An alloy containing 20% tin, balance substantially pure titanium, after 24 hours' anneal at 850° C., has an ultimate strength of 122,000 p. s. i., an elongation in 1" of 12%, and a bend ductility of 1.5 T. The fully annealed alloy containing 22.5% tin shows an ultimate strength of 149,000 p. s. i., elongation in 1" of 11%, and a bend ductility of 4.7 T. Bend ductility has diminished, but is still acceptable for most uses.

The foregoing and other properties of typical binary titanium-tin alloys, as fully annealed at 850° C., are tabulated in the following Tables I and II for "iodide" base titanium metal and that of commercial purity, respectively.

TABLE I

Ti-Sn binary alloys (iodide titanium base)  
annealed condition

| Composition,<br>Percent (Balance<br>Titanium), Sn | Tensile Properties: p. s. i. $\times 1,000$ |                                 |                                |                                 |                   |                     |
|---------------------------------------------------|---------------------------------------------|---------------------------------|--------------------------------|---------------------------------|-------------------|---------------------|
|                                                   | 0.2%<br>Offset<br>Yield                     | Ultimate<br>Tensile<br>Strength | Percent<br>Elongation<br>in 1" | Percent<br>Reduction<br>in Area | Min.<br>Bend<br>T | Vickers<br>Hardness |
| 0.....                                            | 27                                          | 43                              | 40                             | 61                              | 0                 | 105                 |
| 1 <sup>2</sup> .....                              | 30                                          | 48                              | 33                             | 56                              | 0                 | 140                 |
| 2.5 <sup>1</sup> .....                            | 50                                          | 69                              | 23                             | 50                              | 0.9               | 217                 |
| 5 <sup>1</sup> .....                              | 56                                          | 73                              | 26                             | 37                              | 1.6               | 235                 |
| 5 <sup>2</sup> .....                              | 45                                          | 64                              | 18                             | 41                              | 2.8               | 208                 |
| 7.5 <sup>1</sup> .....                            | 65                                          | 80                              | 25                             | 40                              | 1.6               | 255                 |
| 10 <sup>3</sup> .....                             | 85                                          | 99                              | 20                             | 36                              | 1.5               | 298                 |
| 10 <sup>2</sup> .....                             | 65                                          | 83                              | 16                             | 34                              | 1.9               | 257                 |
| 12.5 <sup>4</sup> .....                           | 89                                          | 103                             | 18                             | 41                              | 2.5               | 317                 |
| 15 <sup>3</sup> .....                             | 98                                          | 110                             | 19                             | 35                              | 1.5               | 320                 |
| 15 <sup>2</sup> .....                             | 87                                          | 100                             | 13                             | 40                              | 1.8               | 302                 |
| 17.5 <sup>4</sup> .....                           | 103                                         | 111                             | 19                             | 39                              | 1.8               | 340                 |
| 20 <sup>4</sup> .....                             | 117                                         | 122                             | 12                             | 36                              | 1.5               | 324                 |
| 20 <sup>2</sup> .....                             | 115                                         | 118                             | 13                             | 31                              | 1.8               | 337                 |
| 22.5 <sup>4</sup> .....                           | 135                                         | 149                             | 11                             | 19                              | 4.7               | 339                 |

TABLE II

Ti-Sn binary alloys (commercial purity titanium  
base) annealed condition

| Composition,<br>Percent (Balance<br>Titanium), Sn | Tensile Properties: p. s. i. $\times 1,000$ |                                 |                                |                                 |                     |                   |
|---------------------------------------------------|---------------------------------------------|---------------------------------|--------------------------------|---------------------------------|---------------------|-------------------|
|                                                   | 0.2%<br>Offset<br>Yield                     | Ultimate<br>Tensile<br>Strength | Percent<br>Elongation<br>in 1" | Percent<br>Reduction<br>in Area | Vickers<br>Hardness | Min.<br>Bend<br>T |
| 0.....                                            | 51                                          | 76                              | 21                             | 51                              | 201                 | 0.8               |
| 1.....                                            | 48                                          | 73                              | 21                             | 54                              | 198                 | 0.8               |
| 2.5.....                                          | 67                                          | 88                              | 14                             | 48                              | 236                 | 1.5               |
| 5.....                                            | 71                                          | 90                              | 14                             | 42                              | 246                 | 1.5               |
| 7.5.....                                          | 73                                          | 93                              | 17                             | 45                              | 244                 | 1.6               |
| 10.....                                           | 91                                          | 110                             | 11                             | 36                              | 296                 | 1.5               |
| 12.5.....                                         | 94                                          | 110                             | 12                             | 38                              | 300                 | 2.2               |
| 15.....                                           | 108                                         | 123                             | 10                             | 35                              | 313                 | 2.3               |
| 16 <sup>1</sup> .....                             | 97                                          | 115                             | 9                              | 12                              | 303                 | 1.4               |
| 17.5.....                                         | 110                                         | 121                             | 12                             | 36                              | 340                 | 2.2               |
| 19 <sup>1</sup> .....                             | 93                                          | 121                             | 12                             | 18                              | 330                 | 1.8               |
| 20.....                                           | 123                                         | 131                             | 10                             | 39                              | 330                 | 2.2               |
| 22.5.....                                         | 139                                         | 150                             | 5                              | 19                              | 341                 | 2.2               |

<sup>1</sup> Annealed at 950° C.; other analyses annealed at 850° C.

The alloys of this invention are characterized by an unusual tolerance for the interstitial contaminants, oxygen, nitrogen and carbon. The addition of one or more of these interstitial components in amounts substantially greater than those usable in other titanium alloys has a pronounced strengthening effect with a relatively small loss of ductility. Moreover, the tolerance for oxygen and nitrogen remains substantially the same over a broad range of tin content. For 10

example, alloys of titanium with up to at least 15% tin, may contain as much as 0.3% nitrogen and still possess a ductility adequate for the most exacting of all uses, viz. sheet which is stretched in fabricating to finished form. The effects of controlled and progressively increasing additions of these interstitials to the binary alloys of Tables I and II are shown in the following Tables III and IV, respectively.

TABLE III  
Ti-Sn alloys containing interstitial additions  
(iodide titanium base) anneal condition

| Composition, Percent<br>(Balance Titanium) |      |      |    | Tensile Properties: p. s. i. $\times 1,000$ |                      |                                |                                 |                     |                   |
|--------------------------------------------|------|------|----|---------------------------------------------|----------------------|--------------------------------|---------------------------------|---------------------|-------------------|
| Sn                                         | C    | O    | N  | 0.2% Off-<br>set Yield                      | Ultimate<br>Strength | Percent<br>Elongation<br>in 1" | Percent<br>Reduction<br>in Area | Vickers<br>Hardness | Min.<br>Bend<br>T |
| 0                                          | --   | --   | -- | 27                                          | 43                   | 40                             | 61                              | 105                 | 0                 |
| 1                                          | 0.1  | --   | -- | 46                                          | 59                   | 34                             | 52                              | 180                 | 0.5               |
| 1                                          | 0.2  | --   | -- | 55                                          | 70                   | 28                             | 48                              | 205                 | 0                 |
| 2.5                                        | 0.1  | --   | -- | 55                                          | 66                   | 31                             | 55                              | 220                 | 0.5               |
| 2.5                                        | 0.2  | --   | -- | 65                                          | 74                   | 29                             | 51                              | 235                 | 0.5               |
| 5                                          | 0.1  | --   | -- | 65                                          | 74                   | 26                             | 57                              | 239                 | 0.5               |
| 5                                          | 0.2  | --   | -- | 79                                          | 83                   | 29                             | 53                              | 265                 | 0.5               |
| 5                                          | 0.4  | --   | -- | 92                                          | 99                   | 24                             | 51                              | 290                 | 0                 |
| 5                                          | 0.5  | --   | -- | 109                                         | 117                  | 24                             | 43                              | 325                 | 1.3               |
| 5                                          | 0.75 | --   | -- | 119                                         | 130                  | 10                             | 14                              | 380                 | 5.8               |
| 5                                          | 1    | --   | -- | 123                                         | 138                  | 7                              | 13                              | 387                 | 8.6               |
| 10                                         | 0.1  | --   | -- | 79                                          | 88                   | 21                             | 57                              | 282                 | 1.0               |
| 10                                         | 0.2  | --   | -- | 97                                          | 102                  | 24                             | 60                              | 303                 | 1.0               |
| 10                                         | 0.4  | --   | -- | 124                                         | 124                  | 14                             | 49                              | 359                 | 0.9               |
| 10                                         | 0.5  | --   | -- | 130                                         | 147                  | 17                             | 51                              | 373                 | 2.1               |
| 10                                         | 0.75 | --   | -- | 164                                         | 164                  | 0                              | 0                               | 433                 | (1)               |
| 15                                         | 0.1  | --   | -- | 93                                          | 104                  | 14                             | 49                              | 302                 | 1.4               |
| 15                                         | 0.2  | --   | -- | 122                                         | 127                  | 11                             | 32                              | 364                 | 1.5               |
| 15                                         | 0.4  | --   | -- | 155                                         | 162                  | 4                              | 34                              | 423                 | 3.6               |
| 1                                          | --   | 0.1  | -- | 49                                          | 67                   | 28                             | 45                              | 208                 | 1.5               |
| 1                                          | --   | 0.2  | -- | 64                                          | 84                   | 25                             | 38                              | 247                 | 2.0               |
| 2.5                                        | --   | 0.1  | -- | 57                                          | 74                   | 26                             | 41                              | 235                 | 1.4               |
| 2.5                                        | --   | 0.2  | -- | 71                                          | 90                   | 24                             | 33                              | 274                 | 2.0               |
| 5                                          | --   | 0.1  | -- | 61                                          | 78                   | 23                             | 49                              | 268                 | 1.4               |
| 5                                          | --   | 0.2  | -- | 79                                          | 96                   | 23                             | 47                              | 312                 | 1.0               |
| 5                                          | --   | 0.3  | -- | 102                                         | 113                  | 21                             | 46                              | 365                 | 2.1               |
| 5                                          | --   | 0.4  | -- | 108                                         | 122                  | 12                             | 15                              | 380                 | 6.1               |
| 5                                          | --   | 0.5  | -- | 128                                         | 128                  | 1                              | 10                              | 423                 | 7.6               |
| 10                                         | --   | 0.1  | -- | 81                                          | 94                   | 22                             | 44                              | 319                 | 1.5               |
| 10                                         | --   | 0.2  | -- | 99                                          | 112                  | 16                             | 32                              | 360                 | 1.7               |
| 10                                         | --   | 0.3  | -- | 116                                         | 127                  | 14                             | 40                              | 393                 | 2.1               |
| 10                                         | --   | 0.4  | -- | 131                                         | 138                  | 1                              | 23                              | 410                 | 6.5               |
| 15                                         | --   | 0.1  | -- | 105                                         | 117                  | 14                             | 46                              | 304                 | 2.1               |
| 15                                         | --   | 0.2  | -- | 96                                          | 112                  | 20                             | 45                              | 325                 | 1.7               |
| 15                                         | --   | 0.3  | -- | 124                                         | 134                  | 20                             | 40                              | 380                 | 2.8               |
| 15                                         | --   | 0.5  | -- | 147                                         | 155                  | 11                             | 38                              | 390                 | 3.2               |
| 1                                          | --   | 0.11 | -- | 70                                          | 83                   | 20                             | 40                              | 228                 | 2.0               |
| 1                                          | --   | 0.2  | -- | 94                                          | 105                  | 14                             | 33                              | 310                 | 2.0               |
| 2.5                                        | --   | 0.11 | -- | 75                                          | 90                   | 20                             | 35                              | 258                 | 2.3               |
| 2.5                                        | --   | 0.2  | -- | 100                                         | 109                  | 16                             | 26                              | 332                 | 1.7               |
| 5                                          | --   | 0.06 | -- | 62                                          | 81                   | 23                             | 30                              | 233                 | 2.0               |
| 5                                          | --   | 0.11 | -- | 80                                          | 97                   | 19                             | 29                              | 296                 | 2.0               |
| 5                                          | --   | 0.2  | -- | 107                                         | 115                  | 18                             | 23                              | 366                 | 2.0               |
| 5                                          | --   | 0.29 | -- | 120                                         | 123                  | 20                             | 47                              | 348                 | 2.8               |
| 10                                         | --   | 0.06 | -- | 64                                          | 78                   | 18                             | 50                              | 262                 | 2.2               |
| 10                                         | --   | 0.11 | -- | 88                                          | 100                  | 18                             | 32                              | 297                 | 2.1               |
| 10                                         | --   | 0.18 | -- | 120                                         | 124                  | 13                             | 38                              | 358                 | 1.5               |
| 10                                         | --   | 0.27 | -- | 128                                         | 134                  | 18                             | 46                              | 334                 | 2.2               |
| 15                                         | --   | 0.08 | -- | 81                                          | 89                   | 16                             | 48                              | 310                 | 2.3               |
| 15                                         | --   | 0.13 | -- | 111                                         | 118                  | 17                             | 44                              | 343                 | 1.7               |
| 15                                         | --   | 0.2  | -- | 131                                         | 137                  | 14                             | 36                              | 391                 | 2.2               |
| 15                                         | --   | 0.26 | -- | 144                                         | 151                  | 9                              | 25                              | 387                 | 2.1               |
| 15                                         | --   | 0.3  | -- | 146                                         | 154                  | 12                             | 38                              | 397                 | 2.9               |

Brittle.

TABLE IV

Ti-Sn alloys containing interstitial elements  
(commercial purity titanium base) annealed  
condition

| Composition, Percent<br>(Balance Titanium) |      |      |      | Tensile Properties: p. s. i. $\times 1,000$ |                      |                                |                                 |                     |                   |
|--------------------------------------------|------|------|------|---------------------------------------------|----------------------|--------------------------------|---------------------------------|---------------------|-------------------|
| Sn                                         | C    | O    | N    | 0.2% Off-<br>set Yield                      | Ultimate<br>Strength | Percent<br>Elongation<br>in 1" | Percent<br>Reduction<br>in Area | Vickers<br>Hardness | Min.<br>Bend<br>T |
| 0                                          | --   | --   | --   | 51                                          | 76                   | 21                             | 51                              | 201                 | 0.8               |
| 5                                          | 0.1  | --   | --   | 90                                          | 101                  | 25                             | 57                              | 295                 | 1.9               |
| 5                                          | 0.17 | --   | --   | 96                                          | 106                  | 27                             | 61                              | 311                 | 1.8               |
| 5                                          | 0.4  | --   | --   | 113                                         | 121                  | 26                             | 60                              | 335                 | 1.8               |
| 5                                          | 0.54 | --   | --   | 116                                         | 118                  | 27                             | 60                              | 336                 | 1.8               |
| 5                                          | 0.67 | --   | --   | 122                                         | 127                  | 17                             | 46                              | 348                 | 2.0               |
| 5                                          | 0.96 | --   | --   | 121                                         | 129                  | 7                              | 11                              | 367                 | 3.0               |
| 5                                          | --   | 0.1  | --   | 88                                          | 102                  | 20                             | 41                              | 205                 | 1.4               |
| 5                                          | --   | 0.2  | --   | 109                                         | 123                  | 24                             | 53                              | 351                 | 2.5               |
| 5                                          | --   | 0.3  | --   | 128                                         | 141                  | 12                             | 21                              | 392                 | (1)               |
| 5                                          | --   | 0.4  | --   | 137                                         | 148                  | 8                              | 10                              | 403                 | (1)               |
| 5                                          | --   | --   | 0.16 | 105                                         | 117                  | 21                             | 44                              | 335                 | 1.8               |
| 5                                          | --   | --   | 0.28 | 142                                         | 149                  | 12                             | 31                              | 388                 | 7.4               |
| 5                                          | --   | --   | 0.42 | 159                                         | 164                  | 1                              | 8                               | 415                 | (1)               |
| 10                                         | 0.1  | --   | --   | 99                                          | 109                  | 25                             | 58                              | 320                 | 1.8               |
| 10                                         | 0.2  | --   | --   | 112                                         | 118                  | 26                             | 53                              | 356                 | 1.9               |
| 10                                         | 0.43 | --   | --   | 129                                         | 131                  | 27                             | 54                              | 348                 | 2.0               |
| 10                                         | 0.58 | --   | --   | 146                                         | 148                  | 11                             | 32                              | 385                 | 4.5               |
| 10                                         | --   | 0.04 | --   | 96                                          | 108                  | 24                             | 53                              | 324                 | 1.0               |
| 10                                         | --   | 0.2  | --   | 122                                         | 131                  | 19                             | 44                              | 353                 | 2.8               |
| 10                                         | --   | 0.3  | --   | 115                                         | 128                  | 16                             | 34                              | 376                 | 3.4               |
| 10                                         | --   | 0.4  | --   | 131                                         | 138                  | 16                             | 39                              | 386                 | 3.3               |
| 10                                         | --   | 0.5  | --   | 143                                         | 144                  | 1                              | 8                               | 421                 | (1)               |
| 10                                         | --   | --   | 0.06 | 93                                          | 105                  | 21                             | 48                              | 311                 | 1.8               |
| 10                                         | --   | --   | 0.13 | 114                                         | 124                  | 18                             | 45                              | 337                 | 1.7               |
| 10                                         | --   | --   | 0.34 | 123                                         | 125                  | 3                              | 16                              | 361                 | (1)               |
| 13                                         | 0.1  | --   | --   | 109                                         | 119                  | 19                             | 48                              | 325                 | 3.7               |
| 13                                         | 0.2  | --   | --   | 120                                         | 128                  | 20                             | 52                              | 338                 | 2.7               |
| 13                                         | 0.4  | --   | --   | 141                                         | 149                  | 10                             | 38                              | 357                 | 2.8               |
| 13                                         | 0.56 | --   | --   | 170                                         | 170                  | 3                              | 9                               | 394                 | (1)               |
| 13                                         | --   | 0.1  | --   | 109                                         | 120                  | 19                             | 45                              | 336                 | 1.8               |
| 13                                         | --   | 0.2  | --   | 122                                         | 130                  | 18                             | 38                              | 357                 | 2.4               |
| 13                                         | --   | 0.3  | --   | 127                                         | 137                  | 9                              | 16                              | 387                 | 2.8               |
| 13                                         | --   | 0.4  | --   | 133                                         | 140                  | 18                             | 28                              | 381                 | 5.0               |
| 13                                         | --   | --   | 0.08 | 106                                         | 126                  | 17                             | 40                              | 374                 | 2.5               |
| 13                                         | --   | --   | 0.19 | 143                                         | 150                  | 13                             | 28                              | 412                 | 5.8               |
| 13                                         | --   | --   | 0.24 | 136                                         | 145                  | 16                             | 37                              | 385                 | 2.3               |
| 13                                         | --   | --   | 0.41 | 156                                         | 156                  | 0                              | 6                               | 459                 | (1)               |
| 16                                         | 0.2  | --   | --   | 114                                         | 139                  | 14                             | 27                              | 337                 | 2.1               |
| 16                                         | --   | 0.2  | --   | 109                                         | 137                  | 12                             | 22                              | 341                 | 3.3               |
| 16                                         | --   | --   | 0.18 | 123                                         | 149                  | 9                              | 16                              | 331                 | 6.1               |
| 19                                         | 0.2  | --   | --   | 140                                         | 158                  | 9                              | 15                              | 357                 | 4.0               |
| 19                                         | --   | 0.2  | --   | 120                                         | 140                  | 18                             | 33                              | 339                 | 2.1               |
| 19                                         | --   | --   | 0.14 | 127                                         | 151                  | 5                              | 22                              | 357                 | 4.2               |

<sup>1</sup> Brittle.

From these results it will be observed that additions of tin up to about 23% greatly strengthen the metal while retaining adequate ductility for fabrication purposes, i. e., forging, rolling, etc. For the "iodide" titanium base the yield strength is more than quadrupled from 27,000 to 135,000. p. s. i., while the ultimate strength is more than tripled from 43,000 to 149,000 p. s. i. For any given tin content further strengthening results from controlled additions of one or more of the interstitials. Thus, at the 5% tin level, the addition of 0.5% carbon, approximately doubles the yield and ultimate strength without reducing ductility. Oxygen and nitrogen additions have generally similar effects as shown. The effect of the interstitials in strengthening the titanium-tin alloys in the low tin range of under 2.5% tin is particularly to be emphasized. Thus whereas the Ti-1% Sn binary shows little or no in-

crease in tensile strength as compared to the unalloyed titanium base metal, the further addition of 0.1 or 0.2% of carbon, oxygen or nitrogen increases the ultimate strength by 30% to 150% without noticeable effect in the ductility as compared to the unalloyed titanium base metal. Further increase in the interstitial content further enhances the strength while retaining adequate ductility. In this way the tensile strength of the material may be raised to as much as about 160,000 p. s. i. with retention of adequate ductility as shown, for example, by the 19% tin, 0.2% carbon, commercial purity base analysis.

The alloys of this invention show an unusual behavior with respect to scaling and contamination resistance at forging and rolling temperatures, say temperatures between 900° and 1100° C. Titanium itself and most alloys thereof are

subject to deep penetration by atmospheric gases at these temperatures. For example, when substantially pure titanium is exposed to a temperature of 1000° C. for 2 hours its Knoop hardness number at a depth of 0.012" beneath the surface is increased from about 100 to nearly 300. For alloys of titanium with 5%, 10% or 15% tin, the change in hardness at the surface and at any distance below the surface up to at least 0.012", after a similar high temperature exposure, is negligible. At such temperatures, the tin alloys form a surface scale which flakes off, leaving a fresh surface of essentially the original surface composition and hardness. Troublesome and wasteful "clean-up" after forging is thus obviated. At service temperatures as high as about 425° C., alloys containing up to 20% tin are practically immune to surface oxidation, being in this respect comparable with titanium itself.

In the annexed drawings:

Figs. 1a and 1b illustrate graphically the scaling effects after four hours at 1050° C. in air,

That the alloys of the invention are readily weldable without appreciable loss of ductility is shown by the data in the following Tables V and VI based on arc welding tests in an inert or argon atmosphere.

TABLE V

| Composition, Percent, Bal. Ti<br>(commercial purity) | Minimum Bend<br>Radius T |               |
|------------------------------------------------------|--------------------------|---------------|
|                                                      | Welded                   | Not<br>Welded |
| 1 Sn                                                 | 1.5                      | 0.8           |
| 5 Sn                                                 | 0.2                      | 0.9           |
| 10 Sn                                                | 1.4                      | 1.4           |
| 13 Sn                                                | 0.9                      | 1.4           |
| 15 Sn                                                | 3.4                      | 1.8           |
| 16 Sn                                                | 5.5                      | 1.4           |
| 19 Sn                                                | (1)                      | 1.8           |
| 2Sn-0.13C                                            | 2.2                      | 0.8           |
| 4Sn-0.13C                                            | 2.1                      | 1.4           |
| 7Sn-0.13C                                            | 2.3                      | 1.6           |
| 9.5Sn-0.15C                                          | 4.6                      | 1.8           |
| 10Sn-0.10C                                           | 2.3                      | 2.7           |

<sup>1</sup> Brittle.

TABLE VI

| Composition, percent,<br>Bal. Ti (Commercial<br>purity) | Tensile Properties: p. s. 1.X1,000 |                                |                                 |                      |                                |                                 |
|---------------------------------------------------------|------------------------------------|--------------------------------|---------------------------------|----------------------|--------------------------------|---------------------------------|
|                                                         | Welded                             |                                |                                 | Not Welded           |                                |                                 |
|                                                         | Ultimate<br>Strength               | Percent<br>Elongation<br>in 1" | Percent<br>Reduction<br>in Area | Ultimate<br>Strength | Percent<br>Elongation<br>in 1" | Percent<br>Reduction<br>in Area |
| 2Sn-0.13C                                               | 92                                 | 19                             | 35                              | 100                  | 29                             | 52                              |
| 4Sn-0.13C                                               | 91                                 | 19                             | 29                              | 102                  | 27                             | 52                              |
| 7Sn-0.13C                                               | 101                                | 11                             | 25                              | 114                  | 23                             | 50                              |
| 9.5Sn-0.15C                                             | 115                                | 11                             | 27                              | 138                  | 18                             | 42                              |
| 10Sn-0.10C                                              | 111                                | 10                             | 22                              | 132                  | 16                             | 42                              |

The upper limit for the interstitials for ductile welds are about 0.3% oxygen, about 0.2% nitrogen and about 0.3% carbon.

The alloys may be made by melt casting in a cold mold, employing an electric arc in an inert atmosphere, or may be produced in other ways in which the alloy is rendered molten before casting.

As shown by the data in Tables I-IV inc. the alloys of the invention in general possess ultimate strengths at least 10% in excess of that of the unalloyed titanium base metal, with tensile elongations in general upwards of about 10% and minimum bend ductilities under 9. The vast majority of the alloys of the invention possess ultimate strengths at least 30% to 50% in excess of that of the unalloyed titanium base metal, and this includes the low tin analyses containing one or more of the interstitials in substantial amounts. Where the alloys are to be used in the form of sheets their bend ductilities may range as high as 20 T, and where used in massive form, as in forgings, the tensile elongations may range as low as 1 or 2%. Bend ductility is the minimum radius to which the specimen can be bent through an angle of 75° without fracture, expressed as a multiple of the thickness.

What is claimed is:

1. A ductile titanium base alloy containing: about 5 to 23% tin, up to about 1% carbon, up to about 0.5% oxygen, and up to about 0.3% nitrogen, characterized in having an ultimate strength at least 10% in excess of the unalloyed titanium base metal.

2. A ductile alloy consisting of: about 5 to 23% tin, up to about 1% carbon, up to about 0.5%

nitrogen and oxygen respectively, in terms of metal loss and weight gain respectively, as ordinates, versus tin content, as abscissae, for the binary alloys of the invention.

Figs. 2a-c show graphically the scaling properties and contamination resistance under the conditions above specified of titanium metal of commercial purity; while Figs. 3a-c, 4a-c and 5a-c present corresponding data for the binary Ti-Sn alloys of the present invention for tin contents of 5, 10 and 15%, respectively.

Referring to Figs. 1a and b, it will be observed that the elevated temperature scaling in a nitrogen atmosphere ( $N_2$ ) increases slowly and then more rapidly with increasing tin to a maximum at about 7% tin and drops off thence quite rapidly for higher tin contents. In an oxygen atmosphere ( $O_2$ ) the scaling decreases progressively with increasing tin from a maximum at 0% tin. The curve for scaling in air is substantial a composite of the nitrogen and oxygen graphs, decreasing from a fairly high value at 0% tin to a minimum at about 2.5% tin, rising sharply at upwards of about 5% tin to a maximum at about 7% tin and dropping off rapidly thereafter. As stated the scale formed scales off freely and easily leaving a clean metal surface, this being particularly so in the range of 8 to 16% tin and specifically 10 to 15% tin.

Referring now to Figs. 2a to 5c inc., it will be seen that whereas the unalloyed titanium base metal is subject to deep penetration and accompanying surface hardening by oxygen, nitrogen and atmospheric gases at elevated temperatures, the opposite is true of alloys according to the invention containing upwards of 5% tin.

oxygen, up to about 0.3% nitrogen, and the balance titanium.

3. A ductile titanium base alloy containing: about 5 to 19% tin, up to about 1% carbon, up to about 0.5% oxygen, and up to about 0.3% nitrogen, characterized in having an ultimate strength at least 10% in excess of the unalloyed titanium base metal.

4. A ductile alloy consisting of: about 5 to 19% tin, up to about 1% carbon, up to about 0.5% oxygen, up to about 0.3% nitrogen, and the balance titanium.

5. An alloy consisting essentially of about: 1 to 23% tin, at least one element selected from the group consisting of carbon, oxygen and nitrogen in minimum amount of 0.1% and in maximum amount of 1% for carbon, 0.5% for oxygen, and 0.3% for nitrogen, balance titanium, characterized in having in the annealed condition an ultimate strength at least 30% in excess of the unalloyed titanium base metal, and a minimum bend ductility under 20 T.

6. An alloy consisting essentially of about: 2.5 to 23% tin, at least one element selected from the group consisting of carbon, oxygen and nitro-

5

10

15

20

25

gen in minimum amount of 0.1% and in maximum amount of 1% for carbon, 0.5% for oxygen, and 0.3% for nitrogen, balance titanium, characterized in having in the annealed condition an ultimate strength at least 30% in excess of the unalloyed titanium base metal, and a minimum bend ductility under 20 T.

WALTER L. FINLAY.  
ROBERT I. JAFFEE.  
HORACE R. OGDEN.

## References Cited in the file of this patent

## UNITED STATES PATENTS

| Number    | Name  | Date          |
|-----------|-------|---------------|
| 1,020,515 | Rossi | Mar. 19, 1912 |
| 1,022,598 | Rossi | Apr. 9, 1912  |

## OTHER REFERENCES

Journal of Metals, March 1950, page 498.  
"Research and Development on Titanium Alloys" (part 2), published June 1950 as: AF Technical Report No. 6218, part 2, by U. S. Air Force Air Material Command, Dayton, Ohio.